# EUROPEAN PATENT APPLICATION

(11) **EP 4 389 291 A1**
(43) Date of publication of application: **26.06.2024**
(21) Application number: 22215151.6
(22) Date of filing: 20.12.2022
(51) Int. Cl.: B03D 1/008, B03D 1/01, B03D 1/012

(54) **COLLECTOR COMPOSITION FOR LITHIUM ORE BENEFICIATION**

(71) Applicant: ArrMaz Products Inc., Mulberry, FL 33860 (US)
(72) Inventor: Wang, Guoxin, Lakeland, 33813 (US); Parker, D. Todd, Lakeland, 33813 (US); Gu, Zhengxing, Mulberry, 33860 (US); Wu, Pingkeng, Lakeland, 33813 (US); Gao, Yusheng, Lakeland, 33812 (US); Rasko, Kevin, Lakeland, 33812 (US)
(74) Representative: Arkema Patent

(57) **Abstract**

The invention is related to a collector composition for the beneficiation of lithium containing ores process using an improved collector to upgrade lithium-bearing minerals like but not limited to spodumene. The collector may be a combination of chemicals, comprising: (1) any kind of fatty acids, or derivative fatty acid; (2) an optional fatty acid ester and (3) hydroxamic acids or hydroxamates. The composition may also include amines, preferably water-miscible alkanolamines, as well as sulfonates containing compounds. The composition may also include sodium sulfonate, either natural petroleum sulfonate or synthetic petroleum sulfonate. The collector may further comprise frothers. With the invented collector, the separation efficiency of spodumene from the unwanted impurities can be significantly improved.

## Description

### BACKGROUND OF THE INVENTION

### Cross Reference.

Not Applicable.

### Field of the Invention.

This invention relates generally to a collector composition for the beneficiation of lithium ores. The collector is also suitable for the selective flotation and separation of rare earth metals.

### Description of the Related Art.

Improved beneficiation processes will help with the production of lithium in support of the demand for Li-ion battery operated products. Froth flotation is a widely practiced technique in mineral beneficiation, which is a process where valuable constituents of an ore are concentrated via physical separation. In froth flotation, the valuable minerals (or unwanted gangue materials in reverse flotation) are hydrophobized with the flotation collectors and then attached to the surface of the bubbles to be floated out from the unwanted gangue materials (or valuable minerals in reverse flotation). The ability of the flotation collectors in differentiating the surface hydrophobicity between the valuable minerals and unwanted gangue materials is the key to a successful and efficient froth flotation separation. Since gas bubbles attachment capacity of the different types of minerals in the ore is also important to the separation efficiency, frothers are commonly used in froth flotation and have desirable bubble properties, e.g., bubble stability.
Bubbles with weak stability may have limited capability collecting the solid particles, while bubbles too stable may cause excess foaming affecting the operation efficiency and safety.

Efficient beneficiation of the lithium containing ores such as but not limited to lepidolite, petalite, pegmatite and spodumene is critical for supplying high-grade lithium concentrate to produce lithium-ion batteries. Spodumene, as a pyroxene mineral consisting of lithium aluminum inosilicate with the formula of Li₂O·Al₂O₃·4SiO₂, is an important natural source of lithium. There are many other types of unwanted minerals such as feldspar, mica, carbonate, quartz and iron minerals, which co-exist within the spodumene ore. In order to utilize spodumene ore for lithium production, the grade of spodumene needs to be upgraded with the removal of the undesired impurities.

Froth flotation is an efficient and widely used technique in the beneficiation of ores to isolate the desired element over gangue minerals and may have application for Lithium containing ores especially spodumene. As stated above, the success of flotation separation largely depends on the usage of collectors to differentiate the surface hydrophobicity and gas bubbles attachment capacity of the different types of minerals in the ore. Therefore, the development of collectors is the key for achieving satisfactory separation performance through flotation process.

Collectors for lithium flotation have been disclosed in many patents. US3028008 disclosed fatty acid as flotation collector for obtaining high purity spodumene from beryl. Dispersant and beryl retarding agent like quebracho, sodium sulfide, starch, and lignin sulfonate were used along with the fatty acid collector. US2748938 taught the use of water-insoluble sulfonated oils as collectors for concentrating spodumene. Unsulfonated oils can be used to boost the collecting efficiency of the sulfonated oils. The sulfonated oils include fatty acids and hydrocarbons. US3710934 taught the use of a C9 to C11 aliphatic primary beta-amine for concentrating spodumene ores. The process is a reverse flotation with the siliceous and iron impurities floated away by the claimed collector. CN110369146B described a mixture comprised of sodium hydroxide saponified vegetable oleic acid and dodecyl dimethyl tertiary amine as the spodumene ore flotation collector. CN102600987B disclosed a lithium oxide collector made of oxidized paraffin soap, sulfonated soap, naphthenic acid, and an activation agent. The activation agent is selected from sodium dodecyl sulfate, sodium hexadecanesulfate, or dodecyltrimethylammonium chloride. CN105013620A disclosed a spodumene beneficiation collector comprising of oxidized paraffin wax soap, sodium naphthenate, ethoxylated sodium carboxylates, and quaternary ammonium salt.

Though there are numerous patents on the collectors for lithium flotation, especially from China in the recent years, a few patents involved the use of hydroxamic acid or its salt, which actively chelates with specific minerals for efficient separation. The use of hydroxamic acid or its salt as flotation collectors has been reported in some prior art. US4629556 disclosed the use of alkyl hydroxamate or alkyl hydroxamic acid as collector in removing the colored titaniferous impurities from kaolin clay. US6200377 taught the use of hydroxamate or hydroxamic acid and fatty acid for the selective separation of minerals, which chelate with hydroxamate from the unwanted gangue materials. A silicon-containing compound can be used as conditioner to boost the separation efficiency. US 10478829 described the solution of hydroxamic acid and/or a salt of hydroxamic acid in water-soluble organic solvent as flotation reagents for the beneficiation of oxide and/or sulfide containing ores. The claimed hydroxamic acid is a C6-C22 fatty hydroxamic acid, or a mixture of C8-C12 fatty hydroxamic acid. The patent also taught the method preparing the hydroxamic acid and the salt of the hydroxamic acid. US5237079 claimed a method making alkyl or alkaryl hydroxamic acid and/or salt as collector for the beneficiation of non-sulfide minerals. US7007805 disclosed the fatty hydroxamate with a carbon chain length of 6 to 14 carbon atoms as the froth flotation collector. The collector may also contain less than 1% hydroxylamine and 5% fatty acid. The above patents didn't mention the beneficiation of lithium containing ores.

It is desirable to provide more efficient collectors than those in the prior arts to separate the spodumene from the unwanted impurities.

It is further desirable for the newly developed collector to generate much higher Li₂O concentrate recovery with good selectivity as compared to those commonly used collectors.

### BRIEF DESCRIPTION

The below embodiments and other of the present disclosure will become apparent in light of the following disclosure.

In general, a first embodiment of the invention relates to a collector for beneficiating spodumene ores comprising (a) at least one fatty acid or fatty acid derivative and (b) at least one hydroxamic acid or hydroxamate.

A second embodiment of the invention relates to a collector for beneficiating spodumene ores comprising at least one fatty acid or derivative and at least one fatty acid ester and at least one hydroxamic acid or hydroxamate and optionally an amine, such as but not limited to a fatty (poly)amine, fatty amido (poly)amine, fatty imidazoline, fatty imidazo (poly)amine, fatty (poly) ester amine, fatty (poly) quaternized ammonium salt, an alkanolamine, preferably an alkanolamine, and/or sodium sulfonate. The composition may further comprise at least one frother. In one particular embodiment, the collector may comprise a majority of fatty acids or fatty acid derivatives such as sulfonated fatty acids, or their salts; approximately 0.5% to 20% by weight fatty acid esters; approximately 0.5% to 20% by weight hydroxamic acids or hydroxamates; optionally up to 5%; preferably up to 3% by weight amines; and optionally up to 15% sodium sulfonate. Another optional component may further comprise frothers.

The fatty acid may include 4-22 carbon atoms in the fatty chain and a terminal carboxyl group. Preferred fatty acids may include straight-chain fatty acids, branched chain fatty acids, cyclical molecules containing fatty acids, saturated, unsaturated, aromatic containing fatty acids, fatty acids containing at least one pendant hydroxyl group, preferably containing from 12 to 22 carbon atoms. Examples of sources of the fatty acid include vegetable or animal fats and oils. Tall oil fatty acid (TOFA), Soya fatty acid and canola fatty acid are preferred. Another example of a suitable fatty acid is a ricinoleic acid.

Fatty acid esters are esters that result from the esterification of fatty acids with alcohols. Biodiesels produced by the transesterification of vegetable fats and oils are suitable fatty acid esters. A non-limiting example of constituent fatty acids may be saturated or unsaturated fatty acids, branched chain fatty acids, cyclical containing fatty acids, and aromatic containing fatty acids with 6 to 22 carbon atoms. Examples of suitable alcohols for the esterification or transesterification are methanol, ethanol, butanol, and isopropanol, with methanol being preferred for making the fatty acids methyl esters.

The hydroxamic acids or hydroxamates have the formula

(RC(=O)NH-O)ₙM

where *R* is an alkyl, alkenyl, aryl, alkylaryl or alkenylaryl group having 4 to 24 carbon atoms, preferably 6 to 24 carbon atoms, and M represents hydrogen, alkali metal, or alkaline earth metal with n being the valence of M.

The alkanolamines are a class of chemistry containing both hydroxyl and amino functional groups. The suitable alkanolamines are water-soluble or miscible with water, including but not limiting to aminoethylethanolamine, methanolamine, ethanolamine, N-methylethanolamine, dimethylethanolamine, ethylethanolamine, diethylethanolamine, propylethanolamine, dipropylethanolamine, butylethanolamine, dibutylethanolamine, diethanolamine, methyldiethanolamine, ethyldiethanolamine, propyldiethanolamine, butyldiethanolamine, triethanolamine, isobutanol-2-amine, valinol, alaninol, hydroxyethylpiperazine and combinations thereof. Preferred alkanolamines are aminoethylethanolamine, ethanolamine, methyldiethanolamine, diethanol amine, triethanolamine, hydroxyethylpiperazine and combinations thereof. The alkanolamines may be blended at any ratio.

The fatty (poly)amine, fatty amido (poly)amine, fatty imidazoline, fatty imidazo (poly)amine, fatty (poly) ester amine, fatty (poly) quaternized ammonium salt which may include 4-22 carbon atoms in the fatty chain. Preferred fatty chains may include straight-chains, branched chains, cycles containing chains, saturated, unsaturated, aromatic containing chains, chains with more than 8 carbon atoms containing at least one pendant hydroxyl group, preferably containing from 12 to 22 carbon atoms.

Sodium sulfonates include natural petroleum sulfonate and alkylbenzene derived synthetic petroleum sulfonate with molecular weight from 400 to 600.

The collector may further comprise frothers. Suitable frothers include but not limited to pine oil, methylisobutyl carbinol, alcohols, alkoxylated alcohols, alkoxylated methylisobutylcarbinol and polyglycols, alkoxylated meaning one to hundred, preferably one to sixty, more preferably one to forty repeating alkylene-oxy unit(s) wherein alkylene comprises from one to four carbon atoms in linear or branched chain.

### DETAILED DESCRIPTION OF THE INVENTION

The description herein is merely illustrative of specific manners in which to make and use this invention and are not to be interpreted as limiting in scope. In addition, it is understood that the phraseology and terminology employed herein is for the purpose of description and should not be regarded as limiting.

Unless otherwise defined herein, technical terms used in connection with the present disclosure shall have the meanings that are commonly understood by those of ordinary skill in the art. Further, unless otherwise required by context, singular terms shall include pluralities and plural terms shall include the singular.

All patents, published patent applications, and non-patent publications mentioned in the specification are indicative of the level of skill of those skilled in the art to which the present disclosure pertains. All patents, published patent applications, and non-patent publications referenced in any portion of this application are herein expressly incorporated by reference in their entirety to the same extent as if each individual patent or publication was specifically and individually indicated to be incorporated by reference.

All of the articles and/or methods disclosed herein can be made and executed without undue experimentation in light of the present disclosure. While the articles and methods of the present disclosure have been described in terms of preferred embodiments, it will be apparent to those of ordinary skill in the art that variations can be applied to the articles and/or methods and in the steps or in the sequence of steps of the method(s) described herein without departing from the concept, spirit and scope of the present disclosure. All such similar substitutes and modifications apparent to those skilled in the art are deemed to be within the spirit, scope and concept of the present disclosure.

While the collector compositions have been described with a certain degree of particularity, it is to be noted that many modifications may be made in the details of the components without departing from the spirit and scope of this disclosure. It is understood that the compositions are not limited to the embodiments set forth herein for purposes of exemplification.

The term "at least one" refers to one as well as any quantity more than one, including but not limited to, 1, 2, 3, 4, 5, 10, 15, 20, 30, 40, 50, 100, etc. The term "at least one" can extend up to 100 or 1000 or more depending on the term to which it is attached.

All percentages, parts, proportions, and ratios as used herein are by weight of the total composition, unless otherwise specified. All such weights as they pertain to listed ingredients are based on the active level and therefore do not include solvents or by-products that can be included in commercially available materials, unless otherwise specified.

All references to singular characteristics or limitations of the present invention shall include the corresponding plural characteristics or limitations, and vice-versa, unless otherwise specified or clearly implied to the contrary by the context in which the reference is made.

Numerical ranges as used herein are intended to include every number and subset of numbers contained within that range, whether specifically disclosed or not. Further, these numerical ranges should be construed as providing support for a claim directed to any number or subset of numbers in that range.

As used herein, the words "comprising" (and any form of comprising,
such as "comprise" and "comprises"), "having" (and any form of having, such as "have" and "has"), "including" (and any form of including, such as "includes" and "include") or "containing" (and any form of containing, such as "contains" and "contain") are inclusive or open-ended and do not exclude additional, unrecited elements or method steps. The terms "or combinations thereof' and "and/or combinations thereof' as used herein refer to all permutations and combinations of the listed items preceding the term. For example, "A, B, C, or combinations thereof' is intended to include at least one of: A, B, C, AB, AC, BC, or ABC and, if order is important in a particular context, also BA, CA, CB, CBA, BCA, ACB, BAC, or CAB. Continuing with this example, expressly included are combinations that contain repeats of one or more items or terms, such as BB, AAA, AAB, BBC, AAABCCCC, CBBAAA, CABABB, and so forth. The skilled artisan will understand that typically there is no limit on the number of items or terms in any combination, unless otherwise apparent from the context.

For purposes of the following detailed description, other than in any operating examples, or where otherwise indicated, numbers that express, for example, quantities of ingredients used in the specification and claims are to be understood as being modified in all instances by the term "about". The numerical parameters set forth in the specification and attached claims are approximations that can vary depending upon the desired properties to be obtained in carrying out the invention.

The term "or combinations thereof, "and combinations thereof, and "combinations thereof' as used herein refers to all permutations and combinations of the listed items preceding the term.

In general, the invention relates to a novel collector for use in a flotation process for the beneficiation of lithium containing ores. The collector may be a combination of chemicals, including (1) one or more fatty acids, and/or fatty acids derivatives; (2) one or more hydroxamic acids or hydroxamates, preferably (1) one or more fatty acids, or the derivatives (in one embodiment salts of the fatty acids); (2) one or more fatty acid esters; and (3) one or more hydroxamic acids or hydroxamates. An optional fourth (4) component may be one or more amines, e.g., fatty (poly)amine, fatty amido (poly)amine, fatty imidazoline, fatty imidazo (poly)amine, fatty (poly) ester amine, fatty (poly) quaternized ammonium salt, alkanolamine, sodium sulfonate and combinations thereof. If so desired, the composition may include one or more frothers. These components may be mixed together as one product or may be added separately but preferably at the same time. The separate addition may be either simultaneous or sequential, preferably at the conditioning step prior to flotation. The collector may be emulsified by adding water and suitable emulsifiers before applying to froth flotation.

The composition may include fatty acids, esters of fatty acids and combinations thereof. Preferable fatty acids may include straight-chain fatty acids, branched chain fatty acids, cycle containing fatty acids, saturated, unsaturated, aromatic containing fatty acids containing from 12 to 22 carbon atoms. The fatty acid is not limited to a linear compound; it may be nonlinear. Typical sources for the fatty acids may be vegetable or animal fats and oils. Tall oil fatty acid and canola fatty acid are preferred. The fatty acids may be present in salt form. Preferred amounts of fatty acid/ fatty acid salts included in the composition may range from about 51% to 99% by weight, about 55% to 98% by weight, about 60% to 97% by weight, about 65% to 96% by weight, about 70% to 95% by weight and about 80 to 90% by weight.

Regarding the fatty acid esters, sample constituent fatty acids may be either saturated or unsaturated; preferably they contain 6 to 22 carbon atoms. The hydrocarbon chain of the fatty acids may be linear, branched, cyclic, or aromatic. Suitable alcohols for the esterification or transesterification for making fatty acid esters are methanol, ethanol, butanol, and isopropanol, with methanol being preferred. A concentration of the fatty acid ester in the composition may range from about 1% to 20% by weight, from about 2% to 10% by weight and from more than 2% by weight to less than 10% by weight.

The composition may include hydroxamic acids, hydroxamates and combinations thereof. Examples of non-polar hydrocarbon chains of the hydroxamic acids or hydroxamates are straight or branched C6 to C22 alk(en)yl, aryl or alk(en)ylaryl groups. A concentration of the hydroxamic acids or hydroxamates in the composition may range from about 0.5% to 20% by weight, from about 1% to 10% by weight and from more than about 1.5% by weight to less than 10% by weight.

The composition may inlcude sodium sulfonates, natural petroleum sulfonate or alkylbenzene derived synthetic petroleum sulfonate. A concentration of the sodium sulfonate in the composition may range from 0 to 15% by weight, the afore concentrations are also applicable to the petroleum sulfonate compounds listed above.

The alkanolamines contain both hydroxyl and amino functional groups. Preferably, the alkanolamines may be water soluble or miscible with water with a preference of aminoethylethanolamine, ethanolamine, diethanol amine, methyldiethanolamine, triethanolamine, hydroxyethylpiperazine and combinations thereof. Preferably concentrations of alkanolamines range from more than trace amounts to less than about 5% by weight, preferably less no more than about 3% by weight, even more preferably no more than about 2.5% and even further preferred no more than about 2% by weight.

The fatty (poly)amine, fatty amido (poly)amine, fatty imidazoline, fatty imidazo (poly)amine, fatty (poly) ester amine, fatty (poly) quaternized ammonium salt may include 4-22 carbon atoms in the fatty chain. Preferred fatty chains may include straight-chains, branched chains, cycles containing chains, saturated, unsaturated, aromatic containing chains, chains with more than 8 carbon atoms containing at least one pendant hydroxyl group, preferably containing from 12 to 22 carbon atoms. Preferably concentrations of fatty (poly)amine, fatty amido (poly)amine, fatty imidazoline, fatty imidazo (poly)amine, fatty (poly) ester amine, fatty (poly) quaternized ammonium salt range from more than trace amounts to less than about 5% by weight, preferably less no more than about 3% by weight, even more preferably no more than about 2.5% and even further preferred no more than about 2% by weight.

Frothers can be any commonly used frothers like pine oil, methylisobutyl carbinol, alcohols, alkoxylated alcohols, alkoxylated methylisobutyl carbinol, polyglycols to improve the froth properties such as stability and density, ranging from 0.5 to 5% by weight.

If so desired, the composition may be devoid of an effective amount of silicon to boost separation efficiency.

If so desired, the composition may be devoid of any more than trace amounts of any of alkyne compounds, alkylbenzene compounds and combinations thereof.

If so desired, the composition may be devoid of an effective amount of sulfonated compounds that function as a collector.

If so desired, the composition may be devoid of an effective amount of a separate lithium depressant. An advantage of the disclosed collector is that it may be used to routinely concentrate lithium (Li₂O) from mined spodumene ores having at least about 1% Li₂O into a concentration having at least about 4.5% of Li₂O by a single flotation, preferably greater than about 5.0% and have a recovery of at least about 70% of the Li₂O, preferably greater than about 70%, even more preferably at least about 75%.

A further advantage include that the disclosed collector can improve lithium recovery by more than about 5% over known collectors, preferably about 10% or more.

### ASPECTS

A first aspect of the invention includes a composition (a) at least one fatty acid and/or fatty acid derivative and (b) at least one hydroxamic acid or hydroxamate.

A second aspect of the invention includes a composition comprising: (a) at least one fatty acid and/or fatty acid salt, (b) at least one fatty acid ester and (c) at least one hydroxamic acid or hydroxamate.

In a third aspect the composition of the first or second aspect further comprises at least one amine, sodium sulfonate or a combination of both. One example of a suitable amine is an alkanolamine.

In a fourth aspect the composition of any one of aspects 1 to 3 further comprises a frother.

In a fifth aspect, applicable to anyone of aspects 1-4 wherein a concentration of the fatty acid, fatty acid derivative or the fatty acid salt comprises a majority of the composition by weight.

In a sixth aspect, the composition of anyone of aspects 1-5 comprises up to about 20% by weight of the fatty acid ester and/or the hydroxamic acid or the hydroxamates.

In a seventh aspect, applicable to the composition of anyone of the preceding aspects 1-6 wherein the constituent fatty acid of the fatty acid esters comprises saturated or unsaturated compound with 6 to 22 carbon atoms.

In an eighth aspect, the composition of anyone of aspects 1-7 wherein the hydroxamic acid or hydroxamate has the formula:

(RC(=O)NH-O)ₙM

wherein R is an alkyl, alkenyl, aryl, alkylaryl or alkenylaryl group having 4 to 24 carbon atoms, preferably 6 to 24 carbon atoms, and M represents a hydrogen, alkali metal, or alkaline earth metal with n being charge of valence of M.

In a nineth aspect, the composition of anyone of aspects 1-8 wherein the amine comprises both hydroxyl and amino functional groups and is miscible in water or water soluble.

In a tenth aspect, the composition of anyone of aspects 1-9 wherein the amine comprises at least one selected from the group of aminoethylethanolamine, methanolamine, ethanolamine, diethanolamine, methydiethanolamine, triethanolamine, and aminoethylpiperazine, hydroxyethylpiperazine and combinations thereof.

An eleventh aspect includes a beneficiation process for separating impurities from lithium containing ore. The process includes pulping the ore to produce an ore slurry; reagentizing the ore slurry to produce a reagentized slurry by adding: a collector comprising: (a) at least one fatty acid, fatty acid derivative and combinations thereof, (b) at least one fatty acid ester (c) at least one hydroxamic acid or hydroxamate, (d) at least one amine and optionally a sodium sulfonate. The process may also include separating at least some of the impurities from the lithium and collecting the lithium in the form of a concentrate.

Regarding a twelfth aspect, the reagentizing of the eleventh aspect does not include introducing a separate lithium depressant.

In a thirteenth aspect, applicable to either of aspect 11 or 12, the reagentizing the ore slurry further comprises adding a pH modifier.

In a fourteenth aspect, applicable to anyone of aspects 10-13, the reagentizing further comprises separately adding at least one of (a) the fatty acid or fatty acid derivative (b) the fatty acid ester (c) the hydroxamic acid or hydroxamate or (d) the amine.

In a fifteenth aspect, applicable to anyone of aspects 10-14 the process further comprises combining at least two of (a) the fatty acid or fatty acid derivative, (b) the fatty acid ester (c) the hydroxamic acid or hydroxamate or (d) the alkanolamine prior to being added to the ore slurry.

Aspect sixteenth is a flotation method for removing gangue from lithium containing ores. The method includes producing an ore slurry comprising lithium containing ore and a collector. The collector may comprise (a) at least one fatty acid or fatty acid derivative, (b) at least one fatty acid ester (c) at least one hydroxamic acid or hydroxamate and (d) at least one of an alkanolamine or a sodium sulfonate. The method also includes subjecting the ore slurry to flotation.

In aspect seventeenth, the ore slurry of aspect 16 further comprises a pH modifier.

In aspect eighteenth, applicable to either one of aspects 16 or 17 wherein the subjecting the ore slurry to flotation produces an underflow and an overflow, the method further comprising: separating one of the overflows or the underflow as the gangue; and collecting the other of the underflow or the overflow as lithium concentrate.

In a nineteenth aspect, the composition of any one of aspects 1-15, the composition is used for the beneficiation of a rare earth.

A twentieth aspect a composition comprising (a) at least one fatty acid and/or fatty acid derivative (b) at least one hydroxamic acid or hydroxamate and (c) an amine.

### Examples

The present invention is further illustrated by the following examples. In order that those skilled in the field may better understand how the present invention can be practiced, the following examples are given by way of illustration only and not necessarily by way of limitation. The examples described below share the same procedure for the direct flotation of lithium ores. All the tests were carried out at room temperature. The lithium ores were scrubbed at alkaline pH at 50% solids and then deslimed using 635-mesh sieve. The deslimed slurry was conditioned at 40% solid in 2-liter Denver float cell at 1200 RPM with collector dosage for 5 minutes. After conditioning, the slurry was subject to rougher flotation. The concentrate slurry from the rougher flotation was subject to two cleaner flotation stages in 1-liter Denver float cell. Before each cleaner flotation, the concentrate slurry from the preceding step was conditioned for 30 seconds at 1000 RPM.

### Example I

The spodumene ore sample from Mine A was processed with a collector dosage of 0.3 kg/ton. Compositions of two collectors, a fatty acid collector ("Control") and the invented collector Sample A are shown in Table 1. The flotation performances of two reagents are presented in Table II. It can be found that the invented collector Sample A significantly increased the lithium recovery.

**Table I**

| Components | Control | Sample A |
|---|---|---|
| Fatty acid | 100% | 95% |
| Fatty acid ester | | 2.0% |
| Alkyl Hydroxamic Acid | | 1.7% |
| Alkanolamine | | 0.3% |
| 2-ethylhexanol | | 1.0% |

**Table II**

| Reagent | Dose kg/t | Product | Yield % | Li₂O % | Recovery % |
|---|---|---|---|---|---|
| Control | 0.30 | Concentrate | 10.69 | 5.83 | 63.14 |
| | | Middling 2 | 1.56 | 3.52 | 5.55 |
| | | Middling 1 | 6.15 | 1.18 | 7.35 |
| | | Tail | 81.60 | 0.29 | 23.96 |
| | | Feed | 100.00 | 0.99 | 100.00 |
| Sample A | 0.30 | Concentrate | 11.99 | 5.76 | 71.74 |
| | | Middling 2 | 2.30 | 3.05 | 7.29 |
| | | Middling 1 | 6.51 | 0.91 | 6.16 |
| | | Tail | 79.20 | 0.18 | 14.81 |
| | | Feed | 100.00 | 0.96 | 100.00 |

### Example II

This is the spodumene sample from Mine B. Same procedures were performed as in example 1. The separation results with a fatty acid collector Control and the invented collector Sample A are shown in Table III. That the inventive collector Sample A achieved better performance.

**Table III**

| Reagent | Dose kg/t | Product | Yield % | Li₂O % | Recovery % |
|---|---|---|---|---|---|
| Control | 0.37 | Concentrate | 12.46 | 4.30 | 75.13 |
| | | Middling 2 | 1.10 | 2.66 | 4.11 |
| | | Middling 1 | 3.30 | 1.21 | 5.60 |
| | | Tail | 83.13 | 0.13 | 15.15 |
| | | Feed | 100.00 | 0.71 | 100.00 |
| Sample A | 0.37 | Concentrate | 13.67 | 4.23 | 82.37 |
| | | Middling 2 | 1.41 | 2.55 | 5.10 |
| | | Middling 1 | 4.32 | 0.73 | 4.49 |
| | | Tail | 80.60 | 0.07 | 8.03 |
| | | Feed | 100.00 | 0.70 | 100.00 |

### Example III

In this example, the spodumene sample from Mine C was processed. Compositions of two collectors, a fatty acid collector ("Control") and the invented collector Sample B are shown in Table 4. Same procedures were practiced except that one cleaner flotation was conducted instead of two. For this spodumene feed, high collector dosage was needed. The lab test results show that the invented collector Sample B performed better on Li₂O recovery than the fatty collector Control.

**Table IV**

| Components | Control | Sample B |
|---|---|---|
| Fatty acid | 100% | 80% |
| Sodium sulfonate | | 10% |
| Fatty acid ester | | 2.0% |
| Hydroxamic Acid | | 1.7% |
| Alkanolamine | | 0.3% |
| Polyglycols | | 5.0% |

**Table V**

| Reagent | Dose kg/t | Product | Yield % | Li₂O % | Recovery % |
|---|---|---|---|---|---|
| | | Concentrate | 29.36 | 4.68 | 85.78 |
| Control | 0.60 | Tail | 70.64 | 0.32 | 14.22 |
| | | Feed | 100.00 | 1.60 | 100.00 |
| | | Concentrate | 30.95 | 4.67 | 90.53 |
| Sample B | 0.60 | Tail | 69.05 | 0.22 | 9.47 |
| | | Feed | 100.00 | 1.60 | 100.00 |

## Claims

1. A lithium collector from lithium containing ores comprising: (a) at least one fatty acid, fatty acid derivative and combinations thereof, and (b) at least one hydroxamic acid or hydroxamate.

2. The lithium collector of claim 1 further comprising: at least one fatty acid ester.

3. The collector of either of claim 1 or claim 2 further comprising at least one amine.

4. The collector of anyone of the preceding claims further comprising a frother.

5. The collector of anyone of the preceding claims wherein a concentration of the fatty acid or the fatty acid derivative comprises no more than about 99% by weight and at least about 48% by weight of the collector.

6. The collector of anyone of claims 2-4 wherein the collector comprises up to about 20% by weight of the fatty acid ester and/or the hydroxamic acid or the hydroxamates.

7. The collector of anyone of claims 1-6 wherein the fatty acid comprises more than one of the fatty acids, the fatty acid derivatives and the combinations thereof.

8. The collector of anyone of claims 2-7 wherein a constituent fatty acid of the fatty acid esters comprises saturated or unsaturated compound with 6 to 22 carbon atoms.

9. The collector of anyone of claims 1-8 wherein the hydroxamic acid or hydroxamate has the formula:
(RC(=O)NH-O)ₙM
where R is an alkyl, alkenyl, aryl, alkylaryl or alkenylaryl group having 4 to 24 carbon atoms, preferably 6 to 24 carbon atoms, and M represents a hydrogen, alkali metal, or alkaline earth metal with n being the valence of M

10. The collector of anyone of claims 3-9 wherein the amine comprises both hydroxyl and amino functional groups.

11. The collector of anyone of claims 3-10 wherein the amine comprises at least one selected from the group of a fatty (poly)amine, fatty amido (poly)amine, fatty imidazoline, fatty imidazo (poly)amine, fatty (poly) ester amine, fatty (poly) quaternized ammonium salt, aminoethylethanolamine, methanolamine, ethanolamine, N-methylethanolamine, dimethylethanolamine, ethylethanolamine, diethylethanolamine, propylethanolamine, dipropylethanolamine, butylethanolamine, dibutylethanolamine, diethanolamine, methyldiethanolamine, ethyldiethanolamine, propyldiethanolamine, butyldiethanolamine, triethanolamine, isobutanol-2-amine, valinol, alaninol, hydroxyethylpiperazine and combinations thereof.

12. The collector of anyone of claims 4-11 wherein the frother comprises at least one selected from the group of pine oil, methylisobutyl carbinol, alcohols, alkoxylated alcohols, alkoxylated methylisobutyl carbinol, polyglycols and combinations thereof.

13. The collector of anyone of claims 1-12 wherein the fatty acid or salt comprises a majority of the collector by weight.

14. The collector of anyone of claims 2-13 wherein the fatty acid ester comprises about 0.5% to 20% by weight of the collector.

15. The collector of anyone of claims 1-14 wherein the hydroxamic acid comprises about 0.5% to 20% by weight of the collector.

16. The collector of anyone of claims 1-15 wherein the amine comprises an alkanolamine and up to about 5%, preferably up to 3%, by weight of the collector.

17. The collector of anyone of claims 1-16 wherein the collector comprises an emulsion.

18. The collector of anyone of claims 1-17, wherein
the fatty acid comprises a majority of the collector by weight;
approximately about 0.5% to 10% by weight the fatty acid esters;
approximately about 0.5% to 10% by weight of the hydroxamic acids or hydroxamates; and
approximately about 0.1% to 3% by weight of the alkanolamine.

19. The collector of anyone of claims 1-18 wherein the lithium containing ore comprises spodumene ore.

20. The collector of anyone of claim 1-19 comprising up to about 15 wt. % of a sulfonate containing compound.

21. The collector of claim 20 wherein the sulfonate compound comprises at least one selected from sodium sulfonates, natural petroleum sulfonate, alkylbenzene derived synthetic petroleum sulfonate and combinations thereof.
